# EUROPEAN PATENT APPLICATION

(11) **EP 4 656 759 A1**
(43) Date of publication of application: **03.12.2025**
(21) Application number: 24779616.2
(22) Date of filing: 18.03.2024
(51) Int. Cl.: C22C 38/00, C21D 9/46, C22C 38/14, C22C 38/60, C22C 18/00

(54) **STEEL SHEET, MEMBER, AND METHODS FOR PRODUCING SAME**

(30) Priority: 28.03.2023 JP 2023051053
(71) Applicant: JFE Steel Corporation, Tokyo 100-0011 (JP)
(72) Inventor: TANAKA, Yuji, Tokyo 100-0011 (JP); TOMOZAWA, Masanari, Tokyo 100-0011 (JP); WADA, Yusuke, Tokyo 100-0011 (JP); MINAMI, Hidekazu, Tokyo 100-0011 (JP)
(74) Representative: Hoffmann Eitle
(86) International application number: PCT/JP2024/010397
(87) International publication number: WO 2024/203491

(57) **Abstract**

Provided is a steel sheet and a member having high strength and excellent stretch flangeability and toughness, and methods for producing the same.

A steel sheet has a chemical composition containing, in mass%, C, Si, Mn, P, Al, N, Ti, Nb, and B in specified contents, in which the total area fraction of martensite and bainite is 95% or more, the retained austenite area fraction is 5% or less, the ferrite area fraction is 1% or less, the prior-austenite grain size is 10 µm or less, the C concentration in a prior-austenite grain boundary is equal to or more than 1.5 times the C content in steel, the B concentration in the prior-austenite grain boundary is 0.05% or more in mass%, and the variation in B concentration within the same prior-austenite grain boundary is less than 0.010% in mass%.

## Description

### Technical Field

The present invention relates to a steel sheet, a member, and methods for producing the same.

### Background Art

Automotive steel sheets are required to have strength and excellent stretch flangeability. In addition, high toughness is necessary so that the automotive parts do not fracture upon collision.

Patent Literature 1 discloses a high-strength steel sheet having good workability and a method for producing the same. Patent Literature 2 discloses a high-strength cold rolled steel sheet and a method for producing the same.

### Citation List

### Patent Literature

PTL 1: Japanese Unexamined Patent Application Publication No. 2013-147736
PTL 2: Japanese Unexamined Patent Application Publication No. 2008-106351

### Summary of Invention

### Technical Problem

However, the steel sheets disclosed in Patent Literature 1 and Patent Literature 2 all have a tensile strength TS of less than 1180 MPa, and the stretch flangeability and the toughness are not considered.

The present invention has been made under such circumstances, and an object thereof is to provide a high-strength steel sheet and a member having a tensile strength TS of 1180 MPa or more and excellent stretch flangeability and toughness, and methods for producing the same.

Note that, in the present invention, high strength means that the tensile strength TS as measured in conformity with JIS Z 2241 (2011) is 1180 MPa or more.

In addition, excellent stretch flangeability means that the hole expansion ratio as measured in conformity with JIS Z 2256 (2010) is 30% or more.

Furthermore, excellent toughness means that, in a Charpy impact test performed in conformity with JIS Z 2242 (2018), the brittle-to-ductile transition temperature is - 40°C or lower.

### Solution to Problem

The inventors of the present invention have earnestly conducted studies to achieve the aforementioned object and thus gained following findings.

In order to obtain a tensile strength TS of 1180 MPa or more, the main phase is preferably martensite or bainite. Here, when the area fraction of ferrite is 1% or less, the total area fraction of martensite and bainite is 95% or more, and the area fraction of the retained austenite is 5% or less, void formation at the interfaces between soft ferrite and hard martensite or bainite is suppressed, and the stretch flangeability is improved.

Moreover, addition of Nb decreases the prior-austenite grain size to 10 µm or less, and the toughness is improved. Furthermore, addition of B causes B to segregate to the prior-austenite grain boundaries and strengthen the grain boundaries, thereby improving the toughness.
Meanwhile, even for B-containing steels, some cases have seen moderate improvements in toughness and while others have seen significant improvements in toughness; thus, conditions that have caused the toughness to significantly improve have been investigated in further detail.

It has been found that B segregates nonuniformly to prior-austenite grain boundaries in some cases while B segregates at a uniform concentration in other cases, and that the toughness is significantly improved when B segregates at a uniform concentration. The variation in B concentration within the same prior-austenite grain boundary is focused as the indicator of the uniformity of B segregation, and the toughness has prominently improved when this variation is less than 0.010% in mass%.

Furthermore, a means for causing B to uniformly segregate to the prior-austenite grain boundaries is investigated. As a result, it has been found that, by performing the step of causing B to segregate to the grain boundaries twice, uniform segregation of B occurs. Annealing a cold rolled sheet in an austenite region once causes B to segregate to the austenite grain boundaries; however, at this stage, diffusion of B is insufficient and segregation of B is nonuniform.
Cooling this steel once to form a martensite-bainite microstructure and then annealing the steel again for the second time to form an austenite reverse transformation microstructure. Regarding this point, when retained austenite is present after the first annealing and cooling, an austenite microstructure having the same crystal orientation as in the first annealing is formed from the retained austenite as the nuclei. Furthermore, martensite and bainite contain numerous dislocations, and B that has been dissolved therein diffuses rapidly into austenite grain boundaries through the dislocations during the second annealing; thus, uniform segregation of B occurs. In order to form retained austenite as the nuclei before the second annealing, it is preferable to perform a partial quenching-partitioning treatment after the first annealing to partition carbon into untransformed microstructure to stabilize austenite.

The present invention has been made based on the aforementioned findings. In other words, the gist of features of the present invention is as follows.
[1] A steel sheet having a chemical composition containing, in mass%,
   C: 0.10% or more and 0.30% or less,
   Si: 0.20% or more and 1.20% or less,
   Mn: 2.5% or more and 4.0% or less,
   P: 0.050% or less,
   S: 0.020% or less,
   Al: 0.10% or less,
   N: 0.01% or less,
   Ti: 0.100% or less,
   Nb: 0.002% or more and 0.050% or less,
   B: 0.0015% or more and 0.0040% or less, and
   the balance being Fe and incidental impurities,
      wherein the chemical composition satisfies formula (1) below,
      a total area fraction of martensite and bainite is 95% or more,
      a retained austenite area fraction is 5% or less,
      a ferrite area fraction is 1% or less,
      a prior-austenite grain size is 10 µm or less,
      a C concentration in a prior-austenite grain boundary is equal to or more than 1.5 times a C content in steel,
      a B concentration in the prior-austenite grain boundary is 0.05% or more in mass%,
      a variation in B concentration within the same prior-austenite grain boundary is less than 0.010% in mass%, $\left(\left[%N\right]/14\right) / \left(\left[%Ti\right]/47.9\right) < 1.0$
      in formula (1), [%N] and [%Ti] respectively represent a N content and a Ti content (mass%) in steel.
[2] The steel sheet described in [1], wherein the chemical composition further contains, in mass%, at least one selected from
   V: 0.100% or less,
   Mo: 0.500% or less,
   Cr: 1.00% or less,
   Cu: 1.00% or less,
   Ni: 0.50% or less,
   Sb: 0.200% or less,
   Sn: 0.200% or less,
   Ta: 0.200% or less,
   W: 0.400% or less,
   Zr: 0.0200% or less,
   Ca: 0.0200% or less,
   Mg: 0.0200% or less,
   Co: 0.020% or less,
   REM: 0.0200% or less,
   Te: 0.020% or less,
   Hf: 0.10% or less, and
   Bi: 0.200% or less.
[3] The steel sheet described in [1] or [2], including a coating layer on at least one surface.
[4] A member obtained by using the steel sheet described in any one of [1] to [3].
[5] A method for producing a steel sheet, the method including:
   a hot rolling step of hot-rolling a steel slab having the chemical composition described in [1] or [2] to obtain a hot rolled sheet;
   a pickling step of pickling the hot rolled sheet;
   a cold rolling step of cold-rolling the hot rolled sheet, which has been subjected to the pickling step, to obtain a cold rolled sheet;
   a first annealing step of heating the cold rolled sheet to a first heating temperature equal to or higher than an Ac3 point;
   a cooling step of starting cooling of the cold rolled sheet, which has been subjected to the first annealing step, from the first heating temperature and cooling the cold rolled sheet to a cooling stop temperature equal to or higher than 100°C and lower than an Ms temperature at an average cooling rate of 50°C/s or more;
   a first reheating step of performing heating to a first reheating temperature of 300°C or higher and 400°C or lower after the cooling step, holding the first reheating temperature for 60 s or longer, and performing cooling to room temperature;
   a second annealing step of performing heating to a second heating temperature equal to or higher than an Ac3 point after the first reheating step; and
   a second reheating step of cooling the steel sheet after the second annealing step, heating the steel sheet to a second reheating temperature of 70°C or higher and 200°C or lower, and holding the second reheating temperature for 600 s or longer to obtain a steel sheet.
[6] The method for producing a steel sheet described in [5], further including a coating step of coating the steel sheet after the second annealing step and before the second reheating step.
[7] The method for producing a steel sheet described in [6], further including an alloying step of subjecting the steel sheet to an alloying treatment after the coating step.
[8] A method for producing a member, the method including a step of subjecting the steel sheet described in any one of [1] to [3] to either or both of a forming process and a joining process.

### Advantageous Effects of Invention

According to the present invention, a high-strength steel sheet and a member having a tensile strength TS of 1180 MPa or more and excellent stretch flangeability and toughness, and methods for producing the same can be provided.

### Description of Embodiments

The embodiments of the present invention will now be described. However, the present invention is not limited to the embodiments described below.

A steel sheet according to an embodiment has a chemical composition containing, in mass%, C: 0.10% or more and 0.30% or less, Si: 0.20% or more and 1.20% or less, Mn: 2.5% or more and 4.0% or less, P: 0.050% or less, S: 0.020% or less, Al: 0.10% or less, N: 0.01% or less, Ti: 0.100% or less, Nb: 0.002% or more and 0.050% or less, B: 0.0015% or more and 0.0040% or less, and the balance being Fe and incidental impurities, in which the chemical composition satisfies formula (1) below, a total area fraction of martensite and bainite is 95% or more, a retained austenite area fraction is 5% or less, a ferrite area fraction is 1% or less, a prior-austenite grain size is 10 µm or less, a C concentration in a prior-austenite grain boundary is equal to or more than 1.5 times a C content in steel, a B concentration in the prior-austenite grain boundary is 0.05% or more in mass%, and a variation in B concentration within the same prior-austenite grain boundary is less than 0.010% in mass%. $\left(\left[%N\right]/14\right) / \left(\left[%Ti\right]/47.9\right) < 1.0$

In formula (1), [%N] and [%Ti] respectively represent a N content and a Ti content (mass%) in steel.

### [Chemical composition]

First, appropriate ranges of the chemical composition of the steel sheet and the reasons for the limitations are described. In the description below, "%" indicating the content of a component element in the steel sheet means "mass%" unless clearly indicated otherwise. Unless clearly indicated otherwise, "ppm" means "mass ppm". In this description, a numerical range expressed by using "to" means a range that includes a figure preceding "to" and a figure following "to" as a lower limit value and an upper limit value, respectively.

### C: 0.10% or more and 0.30% or less

C has an effect of strengthening the martensite-bainite microstructure. In addition, C segregates to the prior-austenite grain boundary by the reheating treatment after the second annealing step and has an effect of improving the toughness. At a C content of less than 0.10%, the martensite and bainite area fractions decrease, and a tensile strength TS (hereinafter may also be simply referred to as TS) of 1180 MPa or more is not obtained. Thus, the C content is 0.10% or more. The C content is preferably 0.11% or more.
Meanwhile, at a C content exceeding 0.30%, carboborides of B and iron are formed during annealing, and a sufficient amount of B cannot segregate to the grain boundaries. Thus, the C content is 0.30% or less.
The C content is preferably 0.28% or less.

### Si: 0.20% or more and 1.20% or less

Si is an element effective for solid solution strengthening and the Si content needs to be 0.20% or more. Thus, the Si content is 0.20% or more. The Si content is preferably 0.50% or more.
Meanwhile, the Si is a ferrite-stabilizing element, and ferrite is formed at a Si content exceeding 1.20%, thereby degrading strength, stretch flangeability, and toughness. Thus, the Si content is 1.20% or less. The Si content is preferably 1.10% or less.

### Mn: 2.5% or more and 4.0% or less

Mn is effective for improving hardenability. At a Mn content of less than 2.5%, the martensite and bainite area fractions decrease, and the strength decreases. Thus, the Mn content is 2.5% or more. The Mn content is preferably 2.8% or more.
Meanwhile, at a Mn content exceeding 4.0%, segregation sites become excessively hard, and the toughness is degraded. Thus, the Mn content is 4.0% or less. The Mn content is preferably 3.5% or less.

### P: 0.050% or less

P segregates to the prior-austenite grain boundaries and degrades the toughness; thus, the P content is 0.050% or less. The P content is preferably 0.025% or less. The lower limit of the P content is not particularly specified and may be 0%; however, it involves a higher production cost to make the P content less than 0.001%, and thus the P content is preferably 0.001% or more.

### S: 0.020% or less

S segregates to the prior-austenite grain boundaries and degrades the toughness; thus, the S content is 0.020% or less. The S content is preferably 0.018% or less. The S content is more preferably 0.0040% or less and even more preferably 0.0020% or less.
The lower limit of the S content is not particularly specified; however, it involves a higher production cost to make the S content less than 0.0001%, and thus the S content is preferably 0.0001% or more.

### Al: 0.10% or less

Al is an element that acts as a deoxidizing agent, and, in order to obtain such an effect, the Al content is preferably 0.005% or more. Meanwhile, at an Al content exceeding 0.10%, ferrite tends to form and the strength decreases. Thus, the Al content is 0.10% or less. The Al content is preferably 0.05% or less.

### N: 0.01% or less

N forms nitrides with Nb and B and diminishes the effects of adding Nb and B. Thus, the N content is 0.01% or less. The N content is preferably 0.006% or less. The lower limit is not particularly specified; however, from the production cost perspective, the N content is preferably 0.0001% or more.

### Ti: 0.100% or less

Ti fixes N in the steel as TiN and suppresses formation of BN and NbN, and thus has an effect of enhancing the effects of adding Nb and B and improving the toughness and stretch flangeability. To obtain these effects, the Ti content is preferably 0.005% or more.
Meanwhile, at a Ti content exceeding 0.100%, coarse Ti carbides form on the grain boundaries, and the toughness is degraded. Thus, the Ti content is 0.100% or less. The Ti content is preferably 0.050% or less.

### Nb: 0.002% or more and 0.050% or less

Nb dissolves or precipitates as fine carbides and suppresses growth of the austenite grains during annealing. In addition, Nb can make the crystal grain size finer, complicate the fracture paths, and improve the toughness. In order to obtain such effects, the Nb content is 0.002% or more. The Nb content is preferably 0.005% or more.
Meanwhile, at a Nb content exceeding 0.050%, the effects are saturated, coarse Nb carbides precipitate, and the toughness is degraded. Thus, the Nb content is 0.050% or less. The Nb content is preferably 0.040% or less.

### B: 0.0015% or more and 0.0040% or less

B segregates to the prior-austenite grain boundaries to increase the grain boundary strength and has an effect of improving the toughness. In order to obtain such effects, the B content is 0.0015% or more. The B content is preferably 0.0016% or more.
Meanwhile, at a B content exceeding 0.0040%, carboborides are formed, and the toughness is degraded. Thus, the B content is 0.0040% or less. The B content is preferably 0.0030% or less.$\left(\left[%N\right]/14\right) / \left(\left[%Ti\right]/47.9\right) < 1.0$

In order to obtain the effects of adding B and Nb described above, N, which easily bonds with these elements, needs to be fixed by Ti. For this, the molar fraction of N is to be smaller than the molar fraction of Ti. In other words, the N content and the Ti content in the steel are adjusted to satisfy formula (1) described above. ([%N]/14)/([%Ti]/47.9) is preferably 0.6 or less. Here, in formula (1), [%N] and [%Ti] respectively represent the N content and the Ti content (mass%) in the steel.

The balance other than the aforementioned components is Fe and incidental impurities. Note that, regarding the optional components described below, the effects of the present invention are not impaired as long as the contents thereof are lower than the lower limit values, and thus these optional elements contained in amounts below the lower limits are treated as incidental impurities.

### [Optional components]

The chemical composition of the steel sheet according to this embodiment may further contain, in mass%, at least one element selected from V: 0.100% or less, Mo: 0.500% or less, Cr: 1.00% or less, Cu: 1.00% or less, Ni: 0.50% or less, Sb: 0.200% or less, Sn: 0.200% or less, Ta: 0.200% or less, W: 0.400% or less, Zr: 0.0200% or less, Ca: 0.0200% or less, Mg: 0.0200% or less, Co: 0.020% or less, REM: 0.0200% or less, Te: 0.020% or less, Hf: 0.10% or less, and Bi: 0.200% or less.

### V: 0.100% or less

V forms fine carbides and has an effect of increasing the strength. At a V content exceeding 0.100%, coarse V carbides precipitate, and the toughness is degraded in some cases. Thus, when V is to be contained, the V content is 0.100% or less. The V content is preferably 0.080% or less and more preferably 0.060% or less.
The lower limit of the V content is not particularly limited and may be 0.000%; however, since V has an effect of increasing the strength by forming fine carbides, the V content is preferably 0.001% or more. The V content is more preferably 0.005% or more and even more preferably 0.010% or more.

### Mo: 0.500% or less

Mo improves hardenability and has an effect of increasing the bainite and martensite area fractions. At a Mo content exceeding 0.500%, the effect saturates. Thus, when Mo is to be contained, the Mo content is 0.500% or less. The Mo content is preferably 0.200% or less and more preferably 0.150% or less.
The lower limit of the Mo content is not particularly limited and may be 0.000%; however, since Mo has effects of improving the hardenability and increasing the bainite and martensite area fractions, the Mo content is preferably 0.010% or more. The Mo content is more preferably 0.020% or more and even more preferably 0.030% or more.

### Cr: 1.00% or less

Cr has effects of improving hardenability and increasing the bainite and martensite area fractions. At a Cr content exceeding 1.00%, the effects saturate. Thus, when Cr is to be contained, the Cr content is 1.00% or less. The Cr content is preferably 0.300% or less and more preferably 0.250% or less.
The lower limit of the Cr content is not particularly limited and may be 0.000%; however, since Cr has effects of improving hardenability and increasing the bainite and martensite area fractions, the Cr content is preferably 0.01% or more. The Cr content is more preferably 0.015% or more and even more preferably 0.030% or more.

### Cu: 1.00% or less

Cu, when dissolved, has an effect of increasing the strength. In addition, Cu has an effect of improving the delayed fracture resistance. At a Cu content exceeding 1.00%, grain boundary cracking is likely to occur. Thus, when Cu is to be contained, the Cu content is 1.00% or less. The Cu content is preferably 0.60% or less and more preferably 0.30% or less.
The lower limit of the Cu content is not particularly limited and may be 0.000%; however, since Cu has an effect of increasing the strength when dissolved, the Cu content is preferably 0.01% or more. The Cu content is more preferably 0.02% or more and even more preferably 0.05% or more.

### Ni: 0.50% or less

Ni has an effect of improving the hardenability, but the effect saturates at a Ni content exceeding 0.50%. Thus, when Ni is to be contained, the Ni content is 0.50% or less. The Ni content is preferably 0.20% or less and more preferably 0.15% or less.
The lower limit of the Ni content is not particularly limited and may be 0.00%; however, since Ni has an effect of increasing the hardenability, the Ni content is preferably 0.01% or more. The Ni content is more preferably 0.02% or more and even more preferably 0.03% or more.

### Sb: 0.200% or less

Sb has an effect of suppressing surface oxidation, nitridation, and decarburization of the steel sheet, but the effect saturates at a Sb content exceeding 0.200%. Thus, when Sb is to be contained, the Sb content is 0.200% or less. The Sb content is preferably 0.050% or less and more preferably 0.020% or less.
The lower limit of the Sb content is not particularly limited and may be 0.000%; however, since Sb has an effect of suppressing surface oxidation, nitridation, and decarburization of the steel sheet, the Sb content is preferably 0.001% or more. The Sb content is more preferably 0.002% or more and even more preferably 0.005% or more.

### Sn: 0.200% or less

As with Sb, Sn has an effect of suppressing surface oxidation, nitridation, and decarburization of the steel sheet. At a Sn content exceeding 0.200%, the effect saturates. Thus, when Sn is to be contained, the Sn content is 0.200% or less. The Sn content is preferably 0.050% or less and more preferably 0.020% or less.
The lower limit of the Sn content is not particularly limited and may be 0.000%; however, since Sn has an effect of suppressing surface oxidation, nitridation, and decarburization of the steel sheet, the Sn content is preferably 0.001% or more. The Sn content is more preferably 0.002% or more and even more preferably 0.005% or more.

### Ta: 0.200% or less

Ta forms fine carbides and has an effect of increasing the strength. At a Ta content exceeding 0.200%, coarse Ta carbides precipitate, and the toughness is degraded in some cases. Thus, when Ta is to be contained, the Ta content is 0.200% or less. The Ta content is preferably 0.100% or less and more preferably 0.070% or less.
The lower limit of the Ta content is not particularly limited and may be 0.000%; however, since Ta has an effect of increasing the strength by forming fine carbides, the Ta content is preferably 0.001% or more. The Ta content is more preferably 0.005% or more and even more preferably 0.010% or more.

### W: 0.400% or less

W forms fine carbides and has an effect of increasing the strength. At a W content exceeding 0.400%, coarse W carbides precipitate, and the toughness is degraded in some cases. Thus, when W is to be contained, the W content is 0.400% or less. The W content is preferably 0.300% or less and more preferably 0.250% or less.
The lower limit of the W content is not particularly limited and may be 0.000%; however, since W has an effect of increasing the strength by forming fine carbides, the W content is preferably 0.001% or more. The W content is more preferably 0.005% or more and even more preferably 0.010% or more.

### Zr: 0.0200% or less

Zr has an effect of improving the toughness by spheroidizing inclusions and suppressing the stress concentration. At a Zr content exceeding 0.0200%, a large number of inclusions are formed, and the toughness is degraded in some cases. Thus, when Zr is to be contained, the Zr content is 0.0200% or less. The Zr content is preferably 0.0150% or less and more preferably 0.0100% or less.
The lower limit of the Zr content is not particularly limited and may be 0.0000%; however, since Zr spheroidizes inclusions, suppresses stress concentration, and has an effect of improving the toughness, the Zr content is preferably 0.0001% or more. The Zr content is more preferably 0.0010% or more and even more preferably 0.0020% or more.

### Ca: 0.0200% or less

Ca can be used as a deoxidizing material. At a Ca content exceeding 0.0200%, a large number of Ca-based inclusions are formed, and the toughness is degraded in some cases. Thus, when Ca is to be contained, the Ca content is 0.0200% or less. The Ca content is preferably 0.0100% or less and more preferably 0.0080% or less.
The lower limit of the Ca content is not particularly limited and may be 0.0000%; however, since Ca can be used as a deoxidizing material, the Ca content is preferably 0.0001% or more. The Ca content is more preferably 0.0005% or more and even more preferably 0.0010% or more.

### Mg: 0.0200% or less

Mg can be used as a deoxidizing material. At a Mg content exceeding 0.0200%, a large number of Mg-based inclusions are formed, and the toughness is degraded in some cases. Thus, when Mg is to be contained, the Mg content is 0.0200% or less. The Mg content is preferably 0.0100% or less and more preferably 0.0080% or less.
The lower limit of the Mg content is not particularly limited and may be 0.0000%; however, since Mg can be used as a deoxidizing material, the Mg content is preferably 0.0001% or more. The Mg content is more preferably 0.0005% or more and even more preferably 0.0010% or more.

### Co: 0.020% or less

Co has an effect of increasing the strength through solid solution strengthening. At a Co content exceeding 0.020%, the effect saturates. Thus, when Co is to be contained, the Co content is 0.020% or less. The Co content is preferably 0.015% or less and more preferably 0.010% or less.
The lower limit of the Co content is not particularly limited and may be 0.000%; however, since Co has an effect of increasing the strength through solid solution strengthening, the Co content is preferably 0.001% or more. The Co content is more preferably 0.002% or more and even more preferably 0.005% or more.

### REM: 0.0200% or less

REM has an effect of improving the toughness by spheroidizing inclusions and suppressing the stress concentration. At a REM content exceeding 0.0200%, a large number of inclusions are formed, and the toughness is degraded in some cases. Thus, when REM is to be contained, the REM content is 0.0200% or less. The REM content is preferably 0.0100% or less and more preferably 0.0050% or less.
The lower limit of the REM content is not particularly limited and may be 0.0000%; however, since REM spheroidizes inclusions, suppresses stress concentration, and has an effect of improving the toughness, the REM content is preferably 0.0001% or more. The REM content is more preferably 0.0005% or more and even more preferably 0.0010% or more.

Here, REM refers to a lanthanoid element from scandium (Sc) having atomic number 21 to yttrium (Y) having atonic number 39 and lanthanum (La) having atomic number 57 to lutetium (Lu) having atomic number 71. A REM content is the total content of one or more of the elements selected from among the REMs described above. REM is preferably La, Ce, and Nd.

### Te: 0.020% or less

Te has an effect of improving the toughness by spheroidizing inclusions and suppressing the stress concentration. At a Te content exceeding 0.020%, a large number of inclusions are formed, and the toughness is degraded in some cases. Thus, when Te is to be contained, the Te content is 0.020% or less. The Te content is preferably 0.015% or less and more preferably 0.010% or less.
The lower limit of the Te content is not particularly limited and may be 0.000%; however, since Te spheroidizes inclusions, suppresses stress concentration, and has an effect of improving the toughness, the Te content is preferably 0.001% or more. The Te content is more preferably 0.002% or more and even more preferably 0.004% or more.

### Hf: 0.10% or less

Hf has an effect of improving the toughness by spheroidizing inclusions and suppressing the stress concentration. At a Hf content exceeding 0.10%, a large number of inclusions are formed, and the toughness is degraded. Thus, when Hf is to be contained, the Hf content is 0.10% or less. The Hf content is preferably 0.08% or less and more preferably 0.05% or less.
The lower limit of the Hf content is not particularly limited and may be 0.000%; however, since Hf spheroidizes inclusions, suppresses stress concentration, and has an effect of improving the toughness, the Hf content is preferably 0.01% or more.

### Bi: 0.200% or less.

Bi has an effect of improving bendability by reducing segregation. At a Bi content exceeding 0.200%, a large number of inclusions are formed, and the bendability is degraded in some cases. Thus, when Bi is to be contained, the Bi content is 0.200% or less. The Bi content is preferably 0.100% or less and more preferably 0.050% or less. The Bi content is even more preferably 0.010% or less and even further more preferably 0.005% or less.
The lower limit of the Bi content is not particularly limited and may be 0.000%; however, since Bi has effects of reducing segregation and improve bendability, the Bi content is preferably 0.001% or more. The Bi content is more preferably 0.002% or more and even more preferably 0.003% or more.

### [Steel microstructure]

Next, the steel microstructure of the steel sheet is described.

Total area fraction of martensite and bainite: 95% or more

Martensite and bainite are both hard phases and are necessary for achieving a TS of 1180 MPa or more. Thus, the total area fraction of martensite and bainite is 95% or more. The total area fraction of martensite and bainite is preferably 96% or more. The upper limit of the total area fraction of martensite and bainite is not particularly limited and may be 100%.

### Retained austenite area fraction: 5% or less

Retained austenite may be included as the remaining microstructure other than martensite and bainite. Thus, the retained austenite area fraction is 5% or less. The retained austenite area fraction is preferably 4% or less. The retained austenite area fraction may be 0% or more than 0%.

### Ferrite area fraction: 1% or less

When soft ferrite is present, voids are formed at the interfaces with martensite and bainite constituting the matrix, and the stretch flangeability is degraded; thus, the ferrite area fraction is 1% or less. The ferrite area fraction may be 0%.

The area fraction of each microstructure is measured as follows. The retained austenite area fraction is determined by taking a test specimen from each steel sheet, chemically polishing the rolled surface down to a sheet thickness t/4 position of the steel sheet, measuring the X-ray diffraction intensity and the diffraction peak positions of the polished surface by using an X-ray diffraction (XRD) instrument, and calculating a volume fraction therefrom as the retained austenite area fraction. Next, a sheet thickness section parallel to the rolling direction of each steel sheet is polished and is then etched with 3 vol% nital to prepare an observation surface at the sheet thickness t/4 position. SEM images in three fields of view are taken from the observation surface at a magnification of 2000x with a field of view region of 57.1 µm × 42.9 µm. From the obtained SEM images, the total area fraction of martensite, bainite, and retained austenite, and the area fraction of the microstructure (ferrite) other than martensite, bainite, and retained austenite are determined by image analysis. From the area fraction of the martensite, bainite, and retained austenite obtained by image analysis, the retained austenite area fraction determined by XRD is subtracted to determine the area fraction of martensite and bainite. The average of three fields of view is assumed to be the area fraction of the microstructure.

### Prior-austenite grain size: 10 µm or less

The toughness can be improved by complicating the crack propagation path. In order to obtain this effect, the prior-austenite grain size needs to be 10 µm or less. Thus, the prior-austenite grain size is 10 µm or less. The prior-austenite is preferably 9 µm or less. The lower limit of the prior-austenite grain size is not particularly limited; however, from the viewpoint of production technology, the prior-austenite grain size is preferably 1 µm or more. The prior-austenite grain size is more preferably 2 µm or more and even more preferably 3 µm or more.

Here, the grain size of the prior-austenite is measured as follows. A sheet thickness section parallel to the rolling direction of each steel sheet is polished and then etched with picral to prepare an observation surface. SEM images of the microstructure at the sheet thickness t/4 position in three fields of view are taken from the observation surface with SEM at a magnification of 2000x with a field of view region of 57.1 µm × 42.9 µm. From the obtained microstructure images, the grain size of each of the prior-austenite grains is determined by image analysis, and the average of the three fields of view is assumed to be the prior-austenite grain size (average crystal grain size).

### C concentration in prior-austenite grain boundary: equal to or more than 1.5 times C content in steel

As with B, C segregates to the prior-austenite grain boundaries and thereby strengthens the grain boundaries and improve the toughness. The aforementioned effect is obtained as long as the C concentration in the prior-austenite grain boundary is equal to or more than 1.5 times the C content in the steel. Thus, the C concentration in the prior-austenite grain boundary is equal to or more than 1.5 times the C content in the steel. In other words, the C concentration in the prior-austenite boundary satisfies the following equation. C concentration (mass%) in prior-austenite grain boundary/C content (mass%) in steel ≥ 1.5. The C concentration in the prior-austenite grain boundary is preferably equal to or more than 2.0 times the C content in the steel and more preferably equal to or more than 2.5 times the C content in the steel.
The upper limit of the C concentration in the prior-austenite grain boundary is not specified; however, in order to appropriately prevent precipitation of hard carbides and carboborides on the grain boundary and further improve the toughness, the C concentration is preferably less than 7% in mass%. More preferably, the C concentration is 2% or less in mass%.

### B concentration in prior-austenite grain boundary: 0.05% or more in mass%

B segregates to the prior-austenite grain boundaries and thereby strengthens the grain boundaries, and can improve the toughness. The aforementioned effect is obtained as long as the B concentration in the prior-austenite grain boundary is 0.05% or more in mass%. Thus, the B concentration in the prior-austenite grain boundary is 0.05% or more in mass%. The B concentration in the prior-austenite grain boundary is preferably 0.07% or more and more preferably 0.10% or more in mass%. The upper limit of the B concentration in the prior-austenite grain boundary is not specified; however, in order to appropriately prevent precipitation of hard carboborides on the grain boundary and further improve the toughness, the B concentration is preferably less than 6% in mass%. More preferably, the B concentration is 2% or less in mass%.

### Variation in B concentration within the same prior-austenite grain boundary: less than 0.010% in mass%

In order to improve the toughness, uniformity of the B concentration in the aforementioned grain boundary irrespective of which grain boundary is concerned is critical as well as the aforementioned B concentration in the grain boundary. When the variation is 0.010% or more in mass%, the difference in strength results within a grain boundary, the sites where the B concentration is locally low become prone to cracking, and the toughness improving effect is diminished. Thus, the variation in B concentration within the same prior-austenite grain boundary is less than 0.010% in mass%. The variation is preferably 0.009% or less in mass%, and more preferably 0.008% or less in mass%. The smaller the variation, the better; however, from the viewpoint of the production technology, the variation may be 0.001% or more.

Here, the C concentration, the B concentration, and the variation in the prior-austenite grain boundary are measured as follows. A needle-shaped specimen is prepared from a prior-austenite grain boundary-containing region by SEM-FIB (focused ion beam) method. The obtained needle-shaped specimen is subjected to a 3DAP analysis by using a 3DAP instrument (LEAP 4000X Si produced by AMETEK). The measurement is carried out in laser mode. The specimen temperature is 80 K or lower. The number of C ions and the number of B ions detected from the prior-austenite grain boundary and the number of other ions are used to determine the C concentration and the B concentration in the prior-austenite grain boundary. The average value of two specimens is assumed to be the C concentration or the B concentration. In addition, circular regions not overlapping one another and having a diameter of 5 nm or more and 10 nm or less are set at five sites on a plane of the measured prior-austenite grain boundary, and, for each of the circles, a volume of a column extending in a direction normal to the grain boundary plane is set, the B concentration on the grain boundary is determined for each of the columns, and the standard deviation thereof is assumed to be the variation in B concentration. Note that, in the aforementioned measurement, since the prior-austenite grain size is very large with respect to a region sampled by the SEM-FIB method, the grain boundary targeted by one sampled specimen is from the same grain boundary in all cases. For example, whereas the prior-austenite grain size is about 9 µm, the diameter of the region of the sampled specimen is about 0.1 µm. Thus, the determined variation in B concentration and the like is the variation within the same grain boundary.

According to the present invention, a steel sheet having a tensile strength TS of 1180 MPa or more can be provided. The tensile strength TS of the steel sheet is preferably 1250 MPa or more.

The aforementioned steel sheet may have a coating layer on at least one surface. The coating layer is preferably a hot-dip galvanized layer, a hot-dip galvannealed layer, or an electrogalvanized layer. The composition of the coating layer is not particularly limited and can be any known composition.

The composition of the hot-dip galvanized layer is not particularly limited and may be a common composition. In one example, the coating layer has a composition that contains Fe: 20 mass% or less, Al: 0.001 mass% or more and 1.0 mass% or less, a total of 0 mass% or more and 3.5 mass% or less of at least one selected from the group consisting of Pb, Sb, Si, Sn, Mg, Mn, Ni, Cr, Co, Ca, Cu, Li, Ti, Be, Bi, and REM, and the balance being Zn and incidental impurities.
When the coating layer is a hot-dip galvanized layer, in one example, the Fe content in the coating layer is less than 7 mass%, and when the coating layer is a hot-dip galvannealed layer, in one example, the Fe content in the coating layer is 7 mass% or more and 15 mass% or less and more preferably 8 mass% or more and 13 mass% or less.

The coating weight is not particularly limited and is preferably 20 to 80 g/m² per side of the steel sheet. In one example, the coating layer is formed on both surfaces, top and bottom surfaces, of a steel sheet (a high-strength cold rolled steel sheet).

Next, a method for producing a steel sheet is described.

A method for producing a steel sheet according to an embodiment includes: a hot rolling step of hot-rolling a steel slab having the chemical composition described above to obtain a hot rolled sheet; a pickling step of pickling the hot rolled sheet; a cold rolling step of cold-rolling the hot rolled sheet, which has been subjected to the pickling step, to obtain a cold rolled sheet; a first annealing step of heating the cold rolled sheet to a first heating temperature equal to or higher than an Ac3 point; a cooling step of starting cooling of the cold rolled sheet, which has been subjected to the first annealing step, from the first heating temperature and cooling the cold rolled sheet to a cooling stop temperature equal to or higher than 100°C and lower than an Ms temperature at an average cooling rate of 50°C/s or more; a first reheating step of performing heating to a first reheating temperature of 300°C or higher and 400°C or lower after the cooling step, holding the first reheating temperature for 60 s or longer, and performing cooling to room temperature; a second annealing step of performing heating to a second heating temperature equal to or higher than an Ac3 point after the first reheating step; and a second reheating step of cooling the steel sheet after the second annealing step, heating the steel sheet to a second reheating temperature of 70°C or higher and 200°C or lower, and holding the second reheating temperature for 600 s or longer to obtain a steel sheet.

First, a steel slab having the aforementioned chemical composition is produced.
Here, one example of the steel slab production conditions before the hot rolling step is described. First, a steel material is melted to prepare a molten steel having the aforementioned chemical composition. The melting method is not particularly limited, and any known melting method such as converter melting or electric arc melting is adoptable. The obtained molten steel is solidified to produce a steel slab (slab). The method for producing a steel slab from the molten steel is not particularly limited, and a method such as a continuous casting method, an ingot casting method, or a thin slab casting method can be employed. The steel slab may be temporarily cooled and reheated before hot rolling, or the casted steel slab may be continuously hot-rolled without being cooled to room temperature. The slab heating temperature is preferably 1100°C or higher and preferably 1300°C or lower in view of the rolling load and formation of scale. The slab heating method is not particularly limited, and, for example, the slab may be heated in a heating furnace according to a standard method.

### [Hot rolling step]

The aforementioned steel slab is hot-rolled into a hot rolled sheet. Hot-rolling is not particularly limited, and a common method may be employed. Cooling after the hot rolling is also not particularly limited and the hot rolled sheet is cooled to a coiling temperature. Next, the hot rolled sheet is coiled into a coil. The coiling temperature is preferably 400°C or higher. This is because the hot rolled sheet can be easily coiled without increasing the strength as long as the coiling temperature is 400°C or higher. The coiling temperature is more preferably 550°C or higher. In addition, to appropriately avoid formation of thick scale and improve the yield, the coiling temperature is preferably 750°C or lower. Here, before pickling, the hot rolled sheet may be heat-treated for softening.

### [Pickling step]

After the hot rolling step, the hot rolled sheet is pickled in the pickling step.
In the pickling step, the scale on the hot rolled sheet coiled into a coil can be removed. The method for removing the scale is not particularly limited, but in order to completely remove the scale, pickling is preferably performed while uncoiling the hot rolled coil. The pickling method is not particularly limited and may be any standard method.

### [Cold rolling step]

In a cold rolling step after the pickling step, the hot rolled sheet is cold-rolled into a cold rolled sheet. For example, a hot rolled sheet from which scale has been removed is cleaned as appropriate and then cold-rolled into a cold rolled sheet. The cold rolling method is not particularly limited and may be any standard method.

### [First annealing step: heating to first heating temperature equal to or higher than Ac3 point]

Next, in the first annealing step, the cold rolled sheet is heated to a first heating temperature equal to or higher than the Ac3 point and is annealed in an austenite single phase region. When the first heating temperature is lower than the Ac3 point, ferrite is formed. This ferrite has dislocations reduced by annealing and thus there is no dislocation that serves as a boron (B) diffusion path during the second annealing; thus, it becomes difficult to uniformly segregate boron. Furthermore, excessive heating increases the austenite grain size to larger than 10 µm. Thus, the first heating temperature is equal to or higher than the Ac3 point. The first heating temperature is preferably equal to or higher than Ac3 point + 10°C and more preferably equal to or higher than Ac3 point + 20°C. The austenite microstructure formed by the second annealing has the same crystal structure as the austenite microstructure formed by the first annealing; thus, the first heating temperature is preferably 980°C or lower to make the austenite grain size to 10 µm or less even in the first annealing. The first heating temperature is more preferably 950°C or lower.
The Ac3 point is determined by the following equation. Ac3 (°C) = 881 - 206 × [%C] + 53 × [%Si] - 15 × [%Mn] - 27 × [%Cu] - 20 × [%Ni] - 1 × [%Cr] + 41 × [%Mo] (in this equation, [%M] represents the content (mass%) of the element M in the steel sheet and the value of the element not contained is 0 (zero).)

### [Cooling step: starting cooling from first heating temperature and perform cooling to cooling stop temperature equal to or higher than 100°C and lower than an Ms temperature at average cooling rate of 50°C/s or more]

### [First reheating step: heating to first reheating temperature of 300°C or higher and 400°C or lower, holding first reheating temperature for 60 s or longer, and performing cooling to room temperature]

After the first annealing step, in order to obtain a microstructure in which retained austenite is present at the prior-austenite grain boundaries, the cold rolled sheet is subjected to a partial quenching-partitioning treatment in the cooling step. When the cooling stop temperature of the partial quenching is lower than 100°C, martensite transformation occurs before C partitioning, and a sufficient amount of retained austenite cannot be obtained before the second annealing. When the amount of the retained austenite is insufficient, austenite having a different orientation than that in the first annealing is formed, and it is difficult to have boron (B) uniformly segregate to the grain boundaries of such austenite. Thus, the cooling stop temperature in the cooling step is 100°C or higher. The cooling stop temperature is preferably 120°C or higher and more preferably 150°C or higher. Meanwhile, martensite transformation does not occur at a cooling stop temperature equal to or higher than the Ms temperature, and thus carbon partitioning does not occur during the subsequent reheating and retained austenite is not formed before the second annealing. When the amount of the retained austenite is insufficient, austenite having a different orientation than that in the first annealing is formed, and it is difficult to have boron (B) uniformly segregate to the grain boundaries of such austenite. Thus, the cooling stop temperature in the cooling step is lower than the Ms temperature. The cooling stop temperature is preferably equal to or lower than Ms temperature - 20°C and more preferably equal to or lower than Ms temperature - 30°C.
The Ms temperature is determined by the following equation. Ms (°C) = 499 - 308 × [C] - 10.8 × [Si] - 32.4 × [Mn] - 16.2 × [Ni] - 27 × [Cr] - 10.8 × [Mo] (in this equation, [M] represents a content (mass%) of the element M in the steel sheet, and the value of the element not contained is 0 (zero).

Ferrite transformation occurs when the average cooling rate is less than 50°C/s. This ferrite does not have a specified orientation relationship with austenite, and thus austenite having an orientation different from that in the first annealing is formed in the second annealing, and thus B on the grain boundaries becomes nonuniform. Thus, the average cooling rate is 50°C/s or more. The average cooling rate is preferably 60°C/s or more and more preferably 70°C/s or more.

The upper limit for the average cooling rate is not particularly limited, but the cooling stop temperature becomes difficult to control when the cooling rate is excessively high; thus, the average cooing rate is preferably 1000°C/s or less and more preferably 200°C/s or less.

Note that the average cooling rate (°C/s) in the cooling step is "(first heating temperature (°C)) - (cooling stop temperature (°C))/(cooling time (sec) from first heating temperature (°C) to cooling stop temperature (°C))".

When the first reheating temperature is lower than 300°C, carbon partitioning does not sufficiently occur, and retained austenite is not formed before the second annealing. When the amount of the retained austenite is insufficient, austenite having a different orientation than that in the first annealing is formed, and it is difficult to have boron (B) uniformly segregate to the grain boundaries of such austenite.
Thus, the first reheating temperature is 300°C or higher. The first reheating temperature is preferably 310°C or higher and more preferably 320°C or higher. Meanwhile, when the first reheating temperature exceeds 400°C, non-transformed austenite decomposes into cementite, and retained austenite is not formed before the second annealing. When the amount of the retained austenite is insufficient, austenite having a different orientation than that in the first annealing is formed, and it is difficult to have boron (B) uniformly segregate to the grain boundaries of such austenite. Thus, the first reheating temperature is 400°C or lower. The first reheating temperature is preferably 390°C or lower and more preferably 380°C or lower.

When the time for which the first reheating temperature is held (reheating holding time) is shorter than 60 s, carbon partitioning does not sufficiently occur, and retained austenite is not formed before the second annealing. When the amount of the retained austenite is insufficient, austenite having a different orientation than that in the first annealing is formed, and it is difficult to have boron (B) uniformly segregate to the grain boundaries of such austenite.
Thus, the first reheating temperature holding time is 60 s or longer. The holding time is preferably 80 s or longer and more preferably 100 s or longer.

Meanwhile, although the upper limit of the holding time is not particularly limited, when the holding time is 900 s or longer, non-transformed austenite decomposes into cementite, and austenite is not formed before the second annealing in some cases. Thus, the holding time at the first reheating temperature is preferably shorter than 900 s and more preferably 600 s or shorter.

After holding the first reheating temperature, cooling is performed to room temperature. Here, the room temperature that serves as the cooling stop temperature in the first reheating step is not particularly limited and can be 5 to 50°C.

### [Second annealing step: heating to second heating temperature equal to or higher than Ac3 point]

In the second annealing step, the steel sheet (cold rolled sheet) obtained as above is again heated to a second heating temperature equal to or higher than the Ac3 point and annealed.
During this process, austenite having the same orientation as austenite formed in the first annealing is formed from the retained austenite as the nuclei. As the austenite is formed, boron (B) that has dissolved through the dislocations of martensite before austenite transformation rapidly diffuses into the austenite grain boundaries, and the boron segregation becomes uniform. When the second heating temperature is lower than the Ac3 point, ferrite is formed, and the strength decreases. Thus, the second heating temperature is equal to or higher than the Ac3 point. The second heating temperature is preferably equal to or higher than Ac3 point + 10°C and more preferably equal to or higher than Ac3 point + 20°C.
Meanwhile, excessive heating increases the austenite grain size to over 10 µm and degrades the toughness; thus, the second heating temperature is preferably 980°C or lower. The second heating temperature is more preferably 950°C or lower.

After heating to the second heating temperature, cooling to room temperature may be performed or an overaging treatment may be performed by using the facility in the annealing line in order to perform tempering after formation of a sufficient amount of martensite in the subsequent second reheating step described below.

### [Second reheating step: cooling steel sheet after second annealing step, heating steel sheet to second reheating temperature of 70°C or higher and 200°C or lower, and holding second reheating temperature for 600 s or longer]

In the second reheating step, the steel sheet is cooled after the second annealing step, heated to a second reheating temperature of 70°C or higher and 200°C or lower, and held at the second reheating temperature for 600 s or longer.

The cooling conditions before heating (reheating) here are not particularly limited; however, from the viewpoints of suppressing ferrite transformation and suppressing the strength degradation, cooling is preferably performed at an average cooling rate of 30°C/s or more. Furthermore, cooling is preferably performed to room temperature. Note that the average cooling rate (°C/s) in this step is "(second heating temperature (°C)) - (cooling stop temperature (°C))/(cooling time (sec) from second heating temperature (°C) to cooling stop temperature (°C))".

After cooling, heating (reheating) is performed to the second reheating temperature. Reheating causes C as well as B to segregate to the prior γ grain boundaries and improves the toughness. At a second reheating temperature lower than 70°C, diffusion of C is slow and segregation of C is insufficient. Thus, the second reheating temperature is 70°C or higher. The second reheating temperature is preferably 90°C or higher.
Meanwhile, at a second reheating temperature exceeding 200°C, tempering excessively progresses, carboborides precipitate, the B concentration in the prior-austenite grain boundary cannot be adjusted to 0.05 mass% or more, and the toughness is degraded.
Thus, the second reheating temperature is 200°C or lower. The second reheating temperature is preferably 190°C or lower.

When the holding time at the second reheating temperature (reheating holding time) is shorter than 600 s, diffusion of C is slow and segregation of C is insufficient. Thus, the holding time at the second reheating temperature is 600 s or longer. The holding time at the second reheating temperature is preferably 800 s or longer. The upper limit of the holding time at the second reheating temperature is not particularly limited; however, in order to prevent precipitation of carboborides, the second reheating temperature is preferably 43200 s or shorter (0.5 day or shorter).

### [Coating step and alloying step]

After the aforementioned second annealing step and before the second reheating step, at least one of the surfaces of the steel sheet may be coated in a coating step to obtain a steel sheet (high-strength coated steel sheet). Alternatively, the steel sheet subjected to the coating step (high-strength coated steel sheet) may be heat-treated to alloy the coating layer of the steel sheet and to obtain an alloyed coated steel sheet.

Here, the production conditions other than those described above may be any standard conditions.

A steel sheet according to this embodiment obtained as described above preferably has a sheet thickness of 0.5 mm or more. The sheet thickness is preferably 2.0 mm or less.

### [Member]

In this embodiment, a member that uses the aforementioned steel sheet in at least some part can be provided. In one example, the aforementioned steel sheet may be formed into an intended shape by a pressing process into an automotive part. Here, the automotive part may include, as a raw material, a steel sheet other than the steel sheet of this embodiment. According to this embodiment, since a high-strength steel sheet having a TS of 1180 MPa or more and excellent stretch flangeability and toughness can be provided, a member that has a TS of 1180 MPa or more as well as excellent stretch flangeability and toughness can be provided. The steel sheet according to this embodiment is suitable for use in automotive parts that contribute to weight reduction of automotive bodies. The steel sheet according to this embodiment is particularly suitable for use in, among automotive parts, members that are used in frame structure parts or reinforcing parts in general.

The aforementioned method for producing a member includes a step of subjecting the aforementioned steel sheet to at least one of a forming process or a joining process to obtain a member.

The forming process may involve a common processing method such as pressing without any limitation. The joining process may involve a common welding such as spot welding or arc welding, riveting, crimping, or the like without any limitation.

### EXAMPLES

Steels having chemical compositions shown in Table 1 with the balance being Fe and incidental impurities were melted in a converter to prepare steel slabs. The obtained slabs were reheated, hot-rolled, and coiled to obtain hot rolled coils (hot rolled sheets). Next, the hot rolled coils were pickled while uncoiling, and cold-rolled to obtain cold rolled sheets. The sheet thickness of the hot rolled sheets was 3.0 mm, and the sheet thickness of the cold rolled sheets was 1.2 mm. Annealing (first annealing step, cooling step, first reheating step, and second annealing step) was performed under the conditions shown in Table 2 using a continuous hot-dip galvanizing line to obtain steel sheets (cold rolled steel sheets (CR), hot-dip galvanized steel sheets (GI), and hot-dip galvannealed steel sheets (GA)). The hot-dip galvanized steel sheets were dipped in a coating bath at 460°C, and the coating weight was 35 g/m² per side. Hot-dip galvannealed steel sheets were produced by adjusting the coating amount to 45 g/m² per side and then performing an alloying treatment of holding 520°C for 40 s. The obtained steel sheets except for the steel sheet No. 9 were subjected to a reheating treatment (second reheating step) under the conditions shown in Table 2.

**[Table 1]**

| Steel grade | Chemical composition (mass%) | | | | | | | | | | | |
|---|---|---|---|---|---|---|---|---|---|---|---|---|
| | C | Si | Mn | P | S | Al | N | Ti | Nb | B | other | (N/14)/(Ti/47.9) |
| A | 0.22 | 1.00 | 3.1 | 0.008 | 0.0011 | 0.02 | 0.0020 | 0.021 | 0.036 | 0.0018 | - | 0.33 |
| B | 0.18 | 0.60 | 2.9 | 0.009 | 0.0009 | 0.03 | 0.0018 | 0.015 | 0.028 | 0.0053 | - | 0.41 |
| C | 0.15 | 0.90 | 2.8 | 0.006 | 0.0007 | 0.03 | 0.0031 | 0.026 | 0.040 | 0.0024 | - | 0.41 |
| D | 0.21 | 1.40 | 3.4 | 0.009 | 0.0009 | 0.03 | 0.0030 | 0.025 | 0.030 | 0.0028 | - | 0.41 |
| E | 0.24 | 0.90 | 3.1 | 0.012 | 0.0009 | 0.03 | 0.0025 | 0.021 | 0.031 | 0.0011 | - | 0.41 |
| F | 0.18 | 1.00 | 3.0 | 0.010 | 0.0008 | 0.03 | 0.0022 | 0.028 | 0.021 | 0.0026 | V:0.050 | 0.27 |
| G | 0.23 | 0.90 | 3.2 | 0.006 | 0.0007 | 0.03 | 0.0028 | 0.018 | 0.016 | 0.0023 | Mo:0.100, Cr:0.100 | 0.53 |
| H | 0.17 | 0.80 | 3.5 | 0.011 | 0.0008 | 0.03 | 0.0026 | 0.022 | 0.020 | 0.0019 | Cu:0.20, Ni:0.10 | 0.40 |
| I | 0.18 | 0.80 | 3.1 | 0.004 | 0.0009 | 0.03 | 0.0016 | 0.020 | 0.012 | 0.0021 | Sb:0.010 | 0.27 |
| J | 0.18 | 0.70 | 3.6 | 0.006 | 0.0008 | 0.03 | 0.0031 | 0.018 | 0.031 | 0.0032 | Sn:0.020 | 0.59 |
| K | 0.14 | 0.50 | 3.6 | 0.009 | 0.0011 | 0.03 | 0.0019 | 0.016 | 0.025 | 0.0020 | Ta:0.050, W:0.200 | 0.41 |
| L | 0.12 | 0.60 | 2.8 | 0.008 | 0.0006 | 0.03 | 0.0029 | 0.021 | 0.027 | 0.0024 | Zr:0.0050, Ca:0.0050 | 0.47 |
| M | 0.22 | 0.50 | 3.3 | 0.008 | 0.0005 | 0.03 | 0.0021 | 0.024 | 0.019 | 0.0023 | Mg:0.0050, Co:0.006 | 0.30 |
| N | 0.27 | 0.70 | 3.0 | 0.006 | 0.0008 | 0.03 | 0.0022 | 0.019 | 0.031 | 0.0021 | REM:0.0040, Te:0.005 | 0.40 |
| O | 0.24 | 0.80 | 3.1 | 0.011 | 0.0009 | 0.03 | 0.0022 | 0.023 | 0.020 | 0.0020 | Hf:0.02, Bi:0.004 | 0.33 |
| P | 0.20 | 0.90 | 3.2 | 0.008 | 0.0009 | 0.02 | 0.0069 | 0.018 | 0.040 | 0.0022 | - | 1.31 |
| Q | 0.09 | 1.10 | 3.3 | 0.012 | 0.0012 | 0.02 | 0.0025 | 0.022 | 0.032 | 0.0019 | - | 0.39 |
| R | 0.35 | 0.80 | 2.9 | 0.009 | 0.0009 | 0.03 | 0.0027 | 0.020 | 0.033 | 0.0018 | - | 0.46 |
| S | 0.18 | 0.90 | 2.3 | 0.010 | 0.0011 | 0.02 | 0.0031 | 0.031 | 0.028 | 0.0020 | - | 0.34 |
| T | 0.16 | 0.90 | 3.5 | 0.013 | 0.0013 | 0.03 | 0.0035 | 0.028 | 0.001 | 0.0021 | - | 0.43 |
| U | 0.22 | 1.10 | 2.9 | 0.010 | 0.0012 | 0.03 | 0.0029 | 0.025 | 0.033 | 0.0022 | - | 0.40 |
| v | 0.16 | 0.40 | 2.6 | 0.008 | 0.0011 | 0.02 | 0.0020 | 0.021 | 0.035 | 0.0016 | V:0.095, Mo:0.492, Cr:0.94, Cu:0.96, Ni:0.48, Sb:0.192, Sn:0.194, Ta:0.193, W:0.392, Zr:0.0196, Ca:0.0191, Mg:0.0192, Co:0.017, REM:0.0194, Te:0.016, Hf:0.08, Bi: 0.193 | 0.33 |
| W | 0.20 | 1.00 | 4.1 | 0.006 | 0.0007 | 0.03 | 0.0020 | 0.022 | 0.036 | 0.0018 | - | 0.31 |
| X | 0.21 | 0.90 | 3.2 | 0.054 | 0.0006 | 0.02 | 0.0022 | 0.016 | 0.036 | 0.0018 | - | 0.47 |
| Y | 0.22 | 0.80 | 3.4 | 0.008 | 0.0223 | 0.03 | 0.0024 | 0.022 | 0.036 | 0.0018 | - | 0.37 |
| Z | 0.21 | 0.90 | 3.1 | 0.009 | 0.0012 | 0.12 | 0.0026 | 0.025 | 0.036 | 0.0018 | - | 0.36 |
| AA | 0.20 | 1.00 | 3.2 | 0.006 | 0.0011 | 0.03 | 0.0028 | 0.112 | 0.036 | 0.0018 | - | 0.09 |

| | | | | | | | | | | | | |
|---|---|---|---|---|---|---|---|---|---|---|---|---|
| · The balance of the aforementioned chemical composition is Fe and incidental impurities. · Underlines indicate items outside the scope of the present invention. | | | | | | | | | | | | |

**[Table 2]**

| Steel sheet No. | Steel grade | First annealing | | Cooling | | | First reheating | | | Second annealing | Second reheating | | Coating (*1) |
|---|---|---|---|---|---|---|---|---|---|---|---|---|---|
| | | Ac3 (°C) | First heating temperature (°C) | Ms (°C) | Cooling stop temperature (°C) | Average cooling rate (°C/s) | First reheating temperature (°C) | Reheating holding time (s) | Cooling stop temperature (°C) | Second heating temperature (°C) | Second reheating temperature (°C) | Reheating holding time (s) | |
| 1 | A | 842 | 910 | 320 | 250 | 60 | 350 | 300 | 20 | 910 | 120 | 900 | CR |
| 2 | A | 842 | 820 | 320 | 200 | 60 | 320 | 300 | 20 | 900 | 150 | 1800 | CR |
| 3 | A | 842 | 890 | 320 | 340 | 60 | 380 | 180 | 20 | 890 | 180 | 1800 | CR |
| 4 | A | 842 | 920 | 320 | 200 | 70 | 280 | 400 | 20 | 920 | 150 | 3600 | CR |
| 5 | A | 842 | 910 | 320 | 250 | 70 | 350 | 50 | 20 | 910 | 120 | 1200 | CR |
| 6 | B | 832 | 900 | 343 | 250 | 70 | 350 | 180 | 30 | 900 | 100 | 1500 | CR |
| 7 | C | 856 | 900 | 352 | 250 | 70 | 370 | 120 | 20 | 920 | 90 | 3600 | GA |
| 8 | C | 856 | 900 | 352 | 260 | 60 | 330 | 300 | 20 | 830 | 120 | 2400 | GA |
| 9 | C | 856 | 900 | 352 | 250 | 70 | 370 | 120 | 20 | 920 | - | - | CR |
| 10 | D | 861 | 930 | 309 | 200 | 70 | 350 | 300 | 20 | 920 | 160 | 1500 | GA |
| 11 | E | 833 | 930 | 315 | 200 | 70 | 370 | 300 | 20 | 920 | 180 | 1800 | GA |
| 12 | F | 852 | 930 | 336 | 250 | 70 | 380 | 480 | 30 | 920 | 190 | 1500 | GI |
| 13 | G | 837 | 940 | 311 | 270 | 70 | 330 | 480 | 30 | 910 | 120 | 800 | GI |
| 14 | H | 828 | 920 | 323 | 220 | 70 | 340 | 480 | 30 | 930 | 150 | 3600 | GI |
| 15 | I | 840 | 950 | 334 | 200 | 80 | 330 | 150 | 30 | 950 | 120 | 2400 | GA |
| 16 | J | 827 | 940 | 319 | 150 | 80 | 350 | 100 | 30 | 950 | 90 | 10800 | GA |
| 17 | K | 825 | 940 | 334 | 150 | 80 | 380 | 180 | 30 | 890 | 100 | 3600 | GA |
| 18 | L | 846 | 930 | 365 | 180 | 80 | 370 | 360 | 30 | 900 | 170 | 1800 | GA |
| 19 | M | 813 | 910 | 319 | 250 | 70 | 320 | 420 | 30 | 890 | 150 | 1800 | GA |
| 20 | N | 817 | 880 | 311 | 280 | 60 | 380 | 300 | 30 | 900 | 140 | 2400 | GA |
| 21 | O | 827 | 890 | 316 | 280 | 60 | 370 | 270 | 30 | 880 | 160 | 1200 | GA |
| 22 | P | 840 | 880 | 324 | 280 | 60 | 350 | 300 | 30 | 880 | 150 | 1800 | GA |
| 23 | Q | 871 | 910 | 352 | 200 | 70 | 350 | 300 | 30 | 890 | 100 | 1500 | GA |
| 24 | R | 808 | 860 | 289 | 150 | 70 | 330 | 360 | 30 | 860 | 100 | 1500 | GA |
| 25 | S | 857 | 890 | 359 | 200 | 70 | 330 | 300 | 30 | 880 | 120 | 1800 | GA |
| 26 | T | 843 | 890 | 327 | 180 | 70 | 380 | 360 | 30 | 880 | 160 | 3600 | GA |
| 27 | U | 850 | 900 | 325 | 160 | 70 | 360 | 480 | 30 | 890 | 130 | 2400 | GA |
| 28 | U | 850 | 900 | 325 | 60 | 80 | 330 | 300 | 20 | 880 | 180 | 1200 | GA |
| 29 | U | 850 | 910 | 325 | 150 | 80 | 480 | 480 | 30 | 890 | 160 | 1200 | GA |
| 30 | U | 850 | 900 | 325 | 180 | 70 | 360 | 480 | 30 | 900 | 250 | 3600 | GA |
| 31 | U | 850 | 900 | 325 | 220 | 70 | 350 | 360 | 30 | 910 | 180 | 360 | GA |
| 32 | v | 814 | 900 | 323 | 230 | 70 | 380 | 360 | 20 | 890 | 150 | 1000 | CR |
| 33 | W | 831 | 900 | 294 | 200 | 60 | 340 | 300 | 20 | 910 | 140 | 1200 | CR |
| 34 | X | 837 | 920 | 321 | 220 | 70 | 350 | 400 | 20 | 900 | 160 | 900 | CR |
| 35 | Y | 827 | 910 | 312 | 200 | 80 | 370 | 480 | 20 | 920 | 180 | 1800 | CR |
| 36 | Z | 839 | 930 | 324 | 250 | 70 | 330 | 300 | 20 | 940 | 150 | 2400 | CR |
| 37 | AA | 845 | 920 | 323 | 270 | 60 | 350 | 360 | 20 | 910 | 140 | 3600 | CR |
| 38 | A | 842 | 930 | 320 | 240 | 40 | 360 | 420 | 20 | 940 | 180 | 1800 | CR |

| | | | | | | | | | | | | | |
|---|---|---|---|---|---|---|---|---|---|---|---|---|---|
| · Underlines indicate items outside the scope of the present invention. *1) CR: No coating (cold rolled steel sheet), GA: Hot-dip galvanized steel sheet, GI: hot-dip galvannealed steel sheet | | | | | | | | | | | | | |

For each of obtained steel sheets, the total area fraction of martensite and bainite, the retained austenite area fraction, the ferrite area fraction, the prior-austenite grain size, the C concentration in the prior-austenite grain boundary, the B concentration in the prior-austenite grain boundary, and the variation in B concentration within the same grain boundary of prior-austenite were evaluated according to the methods described above. In addition, the tensile strength TS, the stretch flangeability, and the toughness were evaluated by the methods described below. The results are shown in Table 3.

### [Tensile test]

The obtained steel sheets were subjected to a tensile test in conformity with JIS Z 2241 (2011). A JIS No. 5 test piece for tensile test having a longitudinal direction orienting in a direction orthogonal to the rolling direction was taken, and was subjected to a tensile test to measure the tensile strength (TS). A tensile strength TS of 1180 MPa or more was determined to be good tensile strength.

### [Charpy test]

A Charpy impact test was carried out in conformity with JIS Z 2242 (2018). From each of the obtained steel sheets, a test specimen having a width of 10 mm, a length of 55 mm, and a 90° V notch having a notch depth of 2 mm and being disposed at the lengthwise center was taken such that the direction in which the V notch was formed was perpendicular to the rolling direction of the steel sheet. Subsequently, a Charpy impact test was carried out in a test temperature range of -120 to +120°C. A transition curve was determined from the obtained percent brittle fracture, and the temperature at a percent brittle fracture of 50% was determined to be the brittle-to-ductile transition temperature. Here, the cases where the brittle-to-ductile transition temperature obtained by the Charpy test was -40°C or lower were evaluated as having good toughness. In the tables, the cases where the brittle-to-ductile transition temperature was -40°C or lower are indicated as "excellent" in toughness, and the cases where the brittle-to-ductile transition temperature exceeded -40°C are indicated as "poor" in toughness.

A 100 mm W × 100 m L test specimen was taken from the steel sheet (cold rolled steel sheet or coated steel sheet) and a hole expansion test was conducted in conformity with JIS Z 2256 (2010). A 10 mmφ hole was punched out in a test specimen under the condition of a clearance of 12 ± 1%, a conical punch having a 60° apex angle was elevated to expand hole and stopped as soon as cracks occurred in the sheet thickness direction, and the hole expansion ratio λ was determined from the equation below from the hole diameter after cracking and the hole diameter before the test. Limiting hole expansion ratio: λ (%) = {(Df - D0)/D0} × 100 (in the equation, Df is the hole diameter (mm) at the time cracks occurred and D0 is the initial hole diameter (mm).). Irrespective of the strength of the steel sheet, the cases where the value of λ was 30% or more are determined as having good stretch flangeability.

**[Table 3]**

| Steel sheet No. | Stee grade | M+B area fraction (%) (*1) | RA area fraction (%) (*1) | F area fraction(%) ('1) | Prior γ grain size (µm) (*2) | C concentration ratio (-) (*3) | B concentration (mass%) (*4) | Variation (mass% (*5) | TS (MPa) | λ (%) | Toughness | Reference |
|---|---|---|---|---|---|---|---|---|---|---|---|---|
| 1 | A | 98 | 2 | 0 | 7 | 2.4 | 0.13 | 0.008 | 1521 | 38 | Excellent | Example |
| 2 | A | 98 | 2 | 0 | 6 | 2.3 | 0.12 | 0.025 | 1492 | 32 | Poor | Comparative Example |
| 3 | A | 97 | 3 | 0 | 7 | 2.5 | 0.13 | 0.020 | 1513 | 34 | Poor | Comparative Example |
| 4 | A | 99 | 1 | 0 | 7 | 2.8 | 0.12 | 0.032 | 1506 | 36 | Poor | Comparative Example |
| 5 | A | 98 | 2 | 0 | 6 | 2.1 | 0.12 | 0.030 | 1501 | 38 | Poor | Comparative Example |
| 6 | B | 98 | 2 | 0 | 6 | 2.6 | 0.24 | 0.036 | 1482 | 36 | Poor | Comparative Example |
| 7 | C | 98 | 2 | 0 | 7 | 2.9 | 0.16 | 0.006 | 1328 | 40 | Excellent | Example |
| 8 | C | 91 | 3 | 6 | 5 | 2.4 | 0.11 | 0.013 | 1092 | 25 | Poor | Comparative Example |
| 9 | C | 98 | 2 | 0 | 7 | 1.1 | 0.14 | 0.007 | 1322 | 35 | Poor | Comparative Example |
| 10 | D | 93 | 4 | 3 | 8 | 1.9 | 0.13 | 0.022 | 1156 | 28 | Poor | Comparative Example |
| 11 | E | 96 | 4 | 0 | 8 | 2.3 | 0.03 | 0.005 | 1559 | 33 | Poor | Comparative Example |
| 12 | F | 98 | 2 | 0 | 8 | 2.5 | 0.11 | 0.006 | 1508 | 35 | Excellent | Example |
| 13 | G | 98 | 2 | 0 | 7 | 2.4 | 0.15 | 0.004 | 1535 | 41 | Excellent | Example |
| 14 | H | 99 | 1 | 0 | 8 | 2.6 | 0.13 | 0.008 | 1566 | 38 | Excellent | Example |
| 15 | I | 98 | 2 | 0 | 7 | 2.4 | 0.14 | 0.006 | 1493 | 33 | Excellent | Example |
| 16 | J | 98 | 2 | 0 | 8 | 3.1 | 0.18 | 0.005 | 1489 | 37 | Excellent | Example |
| 17 | K | 99 | 1 | 0 | 6 | 2.3 | 0.12 | 0.005 | 1387 | 34 | Excellent | Example |
| 18 | L | 98 | 2 | 0 | 6 | 2.0 | 0.14 | 0.006 | 1202 | 36 | Excellent | Example |
| 19 | M | 98 | 2 | 0 | 6 | 1.8 | 0.13 | 0.007 | 1528 | 32 | Excellent | Example |
| 20 | N | 98 | 2 | 0 | 7 | 2.2 | 0.13 | 0.005 | 1571 | 35 | Excellent | Example |
| 21 | 0 | 98 | 2 | 0 | 6 | 2.5 | 0.12 | 0.004 | 1538 | 40 | Excellent | Example |
| 22 | P | 99 | 1 | 0 | 12 | 2.4 | 0.03 | 0.004 | 1489 | 32 | Poor | Comparative Example |
| 23 | Q | 65 | 3 | 32 | 8 | 1.7 | 0.10 | 0.005 | 1022 | 28 | Excellent | Comparative Example |
| 24 | R | 96 | 4 | 0 | 7 | 1.9 | 0.04 | 0.008 | 1559 | 31 | Poor | Comparative Example |
| 25 | S | 83 | 3 | 14 | 7 | 2.0 | 0.11 | 0.007 | 1139 | 27 | Excellent | Comparative Example |
| 26 | T | 99 | 1 | 0 | 15 | 2.1 | 0.18 | 0.005 | 1366 | 34 | Poor | Comparative Example |
| 27 | U | 99 | 1 | 0 | 8 | 2.4 | 0.12 | 0.006 | 1509 | 37 | Excellent | Example |
| 28 | U | 99 | 1 | 0 | 7 | 2.1 | 0.11 | 0.033 | 1537 | 31 | Poor | Comparative Example |
| 29 | U | 99 | 1 | 0 | 7 | 2.0 | 0.12 | 0.018 | 1516 | 32 | Poor | Comparative Example |
| 30 | U | 99 | 1 | 0 | 7 | 1.7 | 0.04 | 0.009 | 1488 | 37 | Poor | Comparative Example |
| 31 | U | 99 | 1 | 0 | 7 | 1.3 | 0.12 | 0.008 | 1533 | 32 | Poor | Comparative Example |
| 32 | V | 99 | 1 | 0 | 5 | 2.2 | 0.16 | 0.001 | 1522 | 38 | Excellent | Example |
| 33 | W | 98 | 2 | 0 | 6 | 2.3 | 0.12 | 0.006 | 1577 | 34 | Poor | Comparative Example |
| 34 | X | 99 | 1 | 0 | 8 | 2.1 | 0.14 | 0.008 | 1536 | 32 | Poor | Comparative Example |
| 35 | y | 98 | 2 | 0 | 6 | 2.3 | 0.13 | 0.007 | 1547 | 33 | Poor | Comparative Example |
| 36 | Z | 81 | 4 | 15 | 9 | 2.2 | 0.11 | 0.008 | 1121 | 30 | Excellent | Comparative Example |
| 37 | AA | 99 | 1 | 0 | 8 | 2.6 | 0.14 | 0.006 | 1504 | 31 | Poor | Comparative Example |
| 38 | A | 93 | 2 | 5 | 6 | 2.1 | 0.11 | 0.035 | 1504 | 39 | Poor | Comparative Example |

| | | | | | | | | | | | | |
|---|---|---|---|---|---|---|---|---|---|---|---|---|
| · Underlines indicate items outside the scope of the present invention. *1) M: martensite, B: bainite, RA: retained austenite, F: ferrite *2) Prior γ: Prior-austenite *3) C concentration ratio (concentration ratio: (C concentration (mass%) in prior γ grain boundary/C content (mass%) in steel). *4) B concentration: B concentration (mass%) in prior γ grain boundary. *5) Variation: variation in B concentration within the same prior γ grain boundary. | | | | | | | | | | | | |

Table 3 indicates that the examples of the present invention have a tensile strength TS of 1180 MPa or more and excellent stretch flangeability and toughness. In contrast, in the comparative examples, at least one of the tensile strength TS, the stretch flangeability, and the toughness was poor.

Furthermore, it was found that a member obtained by forming a steel sheet of the example of the present invention, a member obtained by joining the steel sheet, and a member obtained by forming and joining the steel sheet had high strength and excellent stretch flangeability and toughness comparable to those of the steel sheet of the examples of the present invention since the steel sheet of the examples of the present invention had high strength and excellent stretch flangeability and toughness.

## Claims

1. A steel sheet comprising a chemical composition containing, in mass%,
C: 0.10% or more and 0.30% or less,
Si: 0.20% or more and 1.20% or less,
Mn: 2.5% or more and 4.0% or less,
P: 0.050% or less,
S: 0.020% or less,
Al: 0.10% or less,
N: 0.01% or less,
Ti: 0.100% or less,
Nb: 0.002% or more and 0.050% or less,
B: 0.0015% or more and 0.0040% or less, and
the balance being Fe and incidental impurities,
wherein the chemical composition satisfies formula (1) below,
a total area fraction of martensite and bainite is 95% or more,
a retained austenite area fraction is 5% or less,
a ferrite area fraction is 1% or less,
a prior-austenite grain size is 10 µm or less,
a C concentration in a prior-austenite grain boundary is equal to or more than 1.5 times a C content in steel,
a B concentration in the prior-austenite grain boundary is 0.05% or more in mass%, and
a variation in B concentration within the same prior-austenite grain boundary is less than 0.010% in mass%, $\left(\left[%N\right]/14\right) / \left(\left[%Ti\right]/47.9\right) < 1.0$
in formula (1), [%N] and [%Ti] respectively represent a N content and a Ti content (mass%) in steel.

2. The steel sheet according to Claim 1, wherein the chemical composition further contains, in mass%, at least one selected from
V: 0.100% or less,
Mo: 0.500% or less,
Cr: 1.00% or less,
Cu: 1.00% or less,
Ni: 0.50% or less,
Sb: 0.200% or less,
Sn: 0.200% or less,
Ta: 0.200% or less,
W: 0.400% or less,
Zr: 0.0200% or less,
Ca: 0.0200% or less,
Mg: 0.0200% or less,
Co: 0.020% or less,
REM: 0.0200% or less,
Te: 0.020% or less,
Hf: 0.10% or less, and
Bi: 0.200% or less.

3. The steel sheet according to Claim 1 or 2, comprising a coating layer on at least one surface.

4. A member obtained by using the steel sheet according to any one of Claims 1 to 3.

5. A method for producing a steel sheet, the method comprising:
a hot rolling step of hot-rolling a steel slab having the chemical composition according to Claim 1 or 2 to obtain a hot rolled sheet;
a pickling step of pickling the hot rolled sheet;
a cold rolling step of cold-rolling the hot rolled sheet, which has been subjected to the pickling step, to obtain a cold rolled sheet;
a first annealing step of heating the cold rolled sheet to a first heating temperature equal to or higher than an Ac3 point;
a cooling step of starting cooling of the cold rolled sheet, which has been subjected to the first annealing step, from the first heating temperature and cooling the cold rolled sheet to a cooling stop temperature equal to or higher than 100°C and lower than an Ms temperature at an average cooling rate of 50°C/s or more;
a first reheating step of performing heating to a first reheating temperature of 300°C or higher and 400°C or lower after the cooling step, holding the first reheating temperature for 60 s or longer, and performing cooling to room temperature;
a second annealing step of performing heating to a second heating temperature equal to or higher than an Ac3 point after the first reheating step; and
a second reheating step of cooling the steel sheet after the second annealing step, heating the steel sheet to a second reheating temperature of 70°C or higher and 200°C or lower, and holding the second reheating temperature for 600 s or longer to obtain a steel sheet.

6. The method for producing a steel sheet according to Claim 5, further comprising a coating step of coating the steel sheet after the second annealing step and before the second reheating step.

7. The method for producing a steel sheet according to Claim 6, further comprising an alloying step of subjecting the steel sheet to an alloying treatment after the coating step.

8. A method for producing a member, the method comprising a step of subjecting the steel sheet according to any one of Claims 1 to 3 to either or both of a forming process and a joining process.
